

Aug. 24, 1965

J. E. BRIDE  
ELECTROPLATING

3,202,589

Filed Sept. 12, 1963

3 Sheets-Sheet 1



Fig. 1



Fig. 2

INVENTOR.  
JOHN EDWIN BRIDE

BY  
*Hammond & Willard*  
ATTORNEYS

Aug. 24, 1965

J. E. BRIDE

3,202,589

ELECTROPLATING

Filed Sept. 12, 1963

3 Sheets-Sheet 2

Fig. 3



INVENTOR.  
JOHN EDWIN BRIDE

BY

*John Edwin Bride*  
ATTORNEYS

Aug. 24, 1965

J. E. BRIDE

3,202,589

ELECTROPLATING

Filed Sept. 12, 1963

3 Sheets-Sheet 3



Fig. 4

1

3,202,589  
ELECTROPLATING

John Edwin Bride, Mentor, Ohio, assignor to Diamond Alkali Company, Cleveland, Ohio, a corporation of Delaware

Filed Sept. 12, 1963, Ser. No. 306,590  
6 Claims. (Cl. 204—32)

This invention relates to a method of reducing blistering and plating failures on electroplated zinc base die castings and similar articles. Zinc base die castings usually run 90 to 98% zinc with other alloying metals making up the remainder of the composition.

Electroplated zinc base die castings enjoy a large use in fields where mechanical strength of the part is important and the service conditions are severe, such as continued outdoor exposure, and any reduction in service failure will greatly improve the life and acceptance of these products. When used for automotive hardware, kitchen and bathroom hardware, marine hardware, and fixtures and many other fields, electroplated zinc base die castings often develop surface blisters or imperfections which lead to progressive deterioration of the plate and either mar the appearance of the piece or require its replacement long before the object to which it is attached reaches the end of its useful life.

The problem of reducing blistering and improving the life and utility of electroplated zinc base die castings has been before the industry for many years. Thus, F. F. Oplinger in an article entitled "Plating and Heating of Zinc Base Die Castings," Vol. 28, pages 70 to 80 of the Proceedings of the American Electroplaters Society (1940) discusses at length the failure of electroplated zinc based die castings by blistering when subjected to baking at 250° to 350° for the purpose of fixing lacquer coats thereon and recommends as a precaution heating to 225° to 250° F., use of mild anodic electrocleaning, followed by weak acid treatment as the steps to be taken to reduce blistering of electroplated zinc base die casting. However, in spite of these precautions and care taken in the normal production of electroplated zinc base die castings, blistering of the plate and similar failures of the surface of the electroplated metals, and rejects caused thereby, have continued to plague the industry to the present time.

Zinc base die castings are relatively soft and malleable, as compared with copper, brass and ferrous metals and are usually prepared for electroplating by cleaning the grease and dirt from the castings and buffing or polishing to remove burrs, die marks, sprue and ejector pin marks, and other roughness, so that the casting will accept a smooth electroplate. Buffing is usually done with buffing wheels or tumbling barrels or by hand, employing buffing compounds containing abrasives, such as for example, pumice, which are used to facilitate the smoothing of the surfaces of the castings. However, in addition to external protuberances such as burrs, die marks and other roughness, the normal die casting also has pits and depressions below the principal surface thereof, caused by gas pockets or other entraptments within the die. Thus the problem of smoothing the surfaces of the die castings by removal of external protuberances and pits and cavities in a buffing or polishing operation often results in a compromise in which the protuberances are removed and the pits and cavities (sometimes microscopic in size), are covered over by displacement of the surface metal, often with entrapment of buffing compound therein to form a smooth surface which will pass buffing inspection and will accept a smooth electroplate but will lead to subsequent blistering and failure of the electroplate when subjected to severe inspection tests or to baking, or when subjected to normal service conditions over several months.

2

One of the objects of this invention is to provide a relatively certain and inexpensive method of reducing blistering and causes of blistering failures in electroplated zinc base die castings.

5 Another object of this invention is to provide a method for electrolytically modifying the surface characteristics of zinc base die castings and at the same time removing surface oxides, so as to reduce blistering in electroplated articles produced therefrom.

10 Another object of this invention is to provide a process for cleaning and electrolytically modifying the characteristics of zinc base die castings in which unwanted materials lodged in pits and cavities in the surface of the die castings are removed and a clean, continuous surface is presented for acceptance of the subsequently applied electroplate so that the electroplate extends to and covers the bottom of the pits and cavities and does not merely temporarily cover over a pit containing displaced metals, dirt, or buffing compound.

15 20 Another object of this invention is to provide a process for the production of electroplated zinc base die castings, whereby blistering and blistering failures are reduced and a larger percentage of blistering-free and long-life electroplated zinc base die castings are produced.

25 Various other objects and advantages of the invention will become apparent as this description proceeds.

In the accompanying drawings, FIG. 1 is a photomicrograph at a magnification of 500 diameters showing a buffed and plated zinc base die casting with pits containing buffing compound and the surface smoothed over by displaced metal particles so that an apparently satisfactory electroplate is produced.

30 FIG. 2 shows a photomicrograph at a magnification of 250 diameters through a similar casting which has been cleaned with degreasing solvent, anodically treated in a strong alkaline electrolyte for surface modification, and electroplated, by the process of this invention, to provide an electroplate layer extending to the bottom of the pit.

35 40 FIG. 3 is a flow diagram showing a typical illustrative process for producing electroplated zinc base die casting according to a preferred method of practicing this invention, and

45 FIG. 4 is a chart showing the comparative results of a copper accelerated salt spray corrosion test referred to as the CASS test, (more specifically described hereinafter and in "Proceedings of the American Electroplaters Society," 46, page 159 (1959)) the data being taken on seven different classes of electroplated zinc base die castings, some produced under the process of this invention and some by the prior art processes.

50 It will be understood that the processes described herein are illustrative of various methods of practicing the invention but that the invention is not limited to the process herein specifically described, and that although it is primarily useful in preparing electroplated zinc base die castings, it may also be used in the preparation of other electroplated zinc base articles.

55 FIG. 1 illustrates one of the frequent causes of plating failures. This photomicrograph shows (at 500 diameters magnification) a cross-section through the electroplate of an electroplated zinc base die casting, which had been solvent cleaned, buffed, and then electroplated (without anodically treating in an alkaline bath). The points marked "A" represent pits in the original casting, which pits were filled with buffing compound and/or displaced metal and thereafter peened or smoothed over during the buffing operation, pocketing the buffing compound and/or displaced metal but presenting a smooth surface for electroplating and B represents a flaw in the electroplate where traces of the buffing compound or other foreign matter

are visible. In service, or under the more severe physical and chemical inspection tests, the points marked "A" are potential sources of blisters (one or more), and thus failures when subjected to such tests. The original pits were  $\frac{1}{500}$  the size shown in FIG. 1 and would be difficult to identify by visual inspection of the buffed casting.

FIG. 2 illustrates a cross-section at a magnification of 250 diameters through a zinc base die casting which has been subjected to anodic treatment in a strongly alkaline bath, prior to electroplating. In the anodic surface treating operation, the bottom A of the pit has been cleaned out, the edges C of the pit have been rounded off by the anodic electrolytic action, and the copper-nickel electroplate D has been deposited over the bottom as well as the edges of the pit so that there is less chance of blisters developing in the plate in service. The pit in the finished electroplated casting, being less than  $\frac{1}{250}$  the size illustrated, would be barely visible to the naked eye and would not constitute a rejectable flaw in the plated casting. This plated casting would have a long satisfactory service life. The plated casting of FIG. 1 could easily develop blisters within a day or two after plating and jeopardize the reputation of the manufacturer.

While the exact preparation and plating procedure will vary in some details of the method, in different plating plants, and with different types of castings and different end uses therefor, a typical preparation and plating flow diagram is illustrated in FIG. 3, in which block 10 is intended to illustrate that the castings may be cleaned by any of the usual cleaning procedures necessary to remove dirt, mold coating compounds, shopgrease, etc., therefrom, such as the cleaning procedures described in the article by F. F. Oplinger previously referred to. Block 11, shown in dotted lines, is intended to indicate that the casting may or may not be buffed by any of the known buffering procedures, such as buffering wheels, tumbling or the like. Even when buffering is practiced, the buffering time can usually be reduced, as the alkaline anodic electrolytic treating step (block 13) following the buffering and just before the plating operation, does some, if not all of the smoothing accomplished by buffering. Block 12 also shown in dotted lines, is intended to indicate that degreasing by solvents, vapor or other degreasing procedure is an optional but usually desirable precautionary step, although with exceptionally clean castings, the degreasing could conceivably be omitted. The anodic surface treatment in a strong alkaline bath, block 13, described in greater detail hereafter, is essential to get the improved results realized by the practice of this invention, as it cleans off burrs, and protuberances, cleans out pits, rounds off projecting corners and presents a clean surface both on the major surface and within the pits for accepting the electroplated metals. On buffed castings, the usual "touch up" buffering operation, following the main buffering operation, can be omitted, as the anodic surface treatment step in a strong alkaline bath makes further "touch up" buffering unnecessary.

After the anodic surface treatment, the castings must be rinsed free of the alkali and associated zinc salts forming the electrolyte in the anodic surface treating bath, as indicated by block 14, and this is followed by an acid dip for example, in a 0.05 to 1% sulfuric acid solution, if the work-piece is to be electroplated. The block 16 is intended to indicate any of the usual electroplating procedures to cover the exposed surface of the casting with a single or composite layer electroplate as illustrated in the following examples.

In order that those skilled in the art may better understand the principles involved in the present invention, the following specific examples are offered:

#### EXAMPLE 1

For the purpose of illustrating the application and effectiveness of this invention, 280 pieces of zinc base die castings having six different configurations were pre-

pared as noted hereinbelow, electroplated and tested according to the CASS (copper accelerated salt spray) test method (ASTM-Specification B 287-57T) and 210 pieces of zinc base die castings having the same configurations as the CASS test pieces were prepared, as described hereinbelow, electroplated and tested for blistered plate by baking for one hour at 300° F.

The test pieces were divided into seven classes, with 40 pieces in each class for the CASS tests and 30 pieces in each class for the bake test. The classes were prepared for testing by the following method:

| Class        | Buff     | Degrease | Surfaces anodically modified in strongly alkaline bath* | Electroplated |
|--------------|----------|----------|---------------------------------------------------------|---------------|
| Class 1..... | No.....  | Yes..... | Yes; 1.5 min.....                                       | Yes.....      |
| Class 2..... | No.....  | No.....  | Yes, 1.5 min.....                                       | Yes.....      |
| Class 3..... | Yes..... | Yes..... | Yes, 0.75 min.....                                      | Yes.....      |
| Class 4..... | Yes..... | Yes..... | No.....                                                 | Yes.....      |
| Class 5..... | Yes..... | No.....  | Yes, 0.75 min.....                                      | Yes.....      |
| Class 6..... | Yes..... | No.....  | No.....                                                 | Yes.....      |
| Class 7..... | No.....  | No.....  | No.....                                                 | Yes.....      |

\*Bath composition:  
Total NaOH—571 g./l.

Zn—21.0 g./l.  
Temp.—83°-85° F.  
Anode current density—175 to 200 asf.  
Potential—8 volts.

The plating conditions in all instances were controlled as nearly identical as is possible in commercial operations, only the preparation of the article for plating was varied. The plating of the articles, after preparation for plating, consisted of (1) a copper strike; (2) a copper plate; (3) a semi-bright nickel plate; (4) a bright nickel plate, and (5) a chromium plate. Between each of the plating operations, the parts were rinsed, and cleaned, where necessary, and all parts were plated, rinsed clean and replated in the same way. Details of the plating procedure are given hereinbelow.

After plating, the seven classes of plated casting were subjected to the CASS test and the bake test and the results of these tests are illustrated numerically and graphically in FIG. 4. In judging the failures, if more than one small blister, visible to the naked eye, appeared on the part after the test, this part was considered a failure. This test corresponds to an ASTM rating of 9.5 to 10 for acceptable parts.

From FIG. 4 it is clear that at the end of 72 hours of testing by the CASS test, the class 3 casting which had been buffed, degreased and the surfaces anodically treated in a strongly alkaline bath, as noted above, before plating showed fewer failures than any of the other castings, and that the class 1 castings which had been degreased and the surfaces anodically treated in a strongly alkaline bath, noted above, showed the next lowest number of failures. Under the bake test, the class 3 castings also showed up well, and in both tests, the class 7 castings had far too many failures.

The numerical summary of the tests, on the 40 pieces in each of the seven classes for the CASS test, and on the 30 pieces in each of the seven classes for the bake test, is as follows:

TABLE I

| Class        | CASS test data, 40 parts in each class, failures after 72 hours | Bake test data, 30 parts in each class, failures after baking at 300° F. for 1 hour |
|--------------|-----------------------------------------------------------------|-------------------------------------------------------------------------------------|
| Class 1..... | 8.....                                                          | 0.....                                                                              |
| Class 2..... | 11.....                                                         | 4.....                                                                              |
| Class 3..... | 5.....                                                          | 2.....                                                                              |
| Class 4..... | 12.....                                                         | 1.....                                                                              |
| Class 5..... | 11.....                                                         | 1.....                                                                              |
| Class 6..... | 17.....                                                         | 1.....                                                                              |
| Class 7..... | 33.....                                                         | 12.....                                                                             |

As is apparent from Table I and FIG. 4, the castings in class 3, which have been buffed, degreased and anodically treated in a strongly alkaline bath for  $\frac{3}{4}$  of a minute

have fewer failures in the electroplate, and the castings in class 1 (degreased, anodically treated in an alkaline bath, and plated), and in class 5 (buff, anodically treated in an alkaline bath and plated) have the next fewer failures.

## EXAMPLE 2

Zinc base die castings having the composition:

|           | Percent   |
|-----------|-----------|
| Aluminum  | 3.9-4.3   |
| Magnesium | 0.03-0.06 |
| Copper    | maximum   |
| Iron      | do        |
| Lead      | do        |
| Cadmium   | do        |
| Tin       | do        |
| Zinc      | Remainder |

were cleaned by soaking in a proprietary cleaning compound of the commercial alkaline detergent type, jet spraying and rinsing, buffed by the use of high speed buffing wheels, degreased, and anodically treated in a sodium hydroxide-zinc oxide electrolyte containing 655 grams/liter of NaOH, 25 grams of zinc oxide per liter, and 2 grams of basic chromic sulfate per liter, maintained at a temperature of between 80° and 95° F. at an anode current density of 100 to 200 amps./sq. ft. for 3/4 minute. The die castings constituted the anode of the electrolytic cell and magnetite coated cathodes were employed, although other cathodic materials such as platinum, steel, copper and other conductors may be used. The amount of basic chromic sulfate may vary from about 1.5 to 3 grams per liter.

At the end of the anodic surface treating operation, the castings were spray-rinsed and given an acid dip in a 1% by volume sulfuric acid solution and electroplated as follows:

(1) Copper strike: 4 volts, 3 minutes (110° F.)—  
CuCN—4.1 oz./gal.  
Free KCN—1.6 oz./gal.  
pH 12.6

(2) Copper plate: 1.1 volts, 20 minutes (155° F.)—  
CuCN—10.2 oz./gal.  
Free KCN—3.3 oz./gal.  
pH 13.5

Current interruption: 10 sec. on, 3 sec. off.

NOTE: Together with the usual leveling agents, wetting agents and porosity preventing agents.

Thereafter the copper-plated castings were rinsed and cleaned and (3), given a semi-bright nickel plate as follows:

Semi-bright nickel, 26 minutes (135° F.)—  
NiSO<sub>4</sub>·6H<sub>2</sub>O—50 oz./gal.  
NiCl<sub>2</sub>·6H<sub>2</sub>O—6.5 oz./gal.  
H<sub>3</sub>BO<sub>3</sub>—7.0 oz./gal.  
pH—4.0

NOTE: Together with leveling agents, wetting agents and porosity preventing agents.

and after rinsing given (4) a bright nickel plate as follows:

Bright nickel, 13 minutes (155° F.)—  
NiSO<sub>4</sub>·6H<sub>2</sub>O—50 oz./gal.  
NiCl<sub>2</sub>·6H<sub>2</sub>O—8.0 oz./gal.  
H<sub>3</sub>BO<sub>3</sub>—7.0 oz./gal.  
pH—4.0

NOTE: Together with leveling agents, wetting agents and porosity preventing agents.

This was followed by rinsing and (5) chrome plating as follows:

Chrome plate, 5 minutes (115° F.)—  
CrO<sub>3</sub>—50 oz./gal.  
SO<sub>4</sub>—0.28 oz./gal.

This procedure was used to produce the composite electroplate on the castings used in the tests described in Example 1 and in illustrated FIG. 4 and Table I.

## EXAMPLE 3

*Cleaning and electropolishing of unbuffed parts*

Unbuffed zinc base die castings were immersed 2 to 5 minutes in an 8-oz./gal. solution of a commercial line, soak cleaner maintained between 165 and 175° F. for the purpose of cleaning and wetting the surface. After rinsing in hot water followed by cold water, the castings, while still wet, were placed in an 18-gallon electropolishing bath containing 665 g. NaOH/l. and 100 g. ZnO/l., and then electropolished at 300 amp./sq. ft. for the maximum time for obtaining optimum appearance.<sup>1</sup> After being rinsed in hot water, the parts were dipped for about 10 to 20 seconds in a 1 percent by weight sulfuric acid solution. The parts were then rinsed in cold water in preparation for the plating sequence. This is the procedure which was used to prepare the casting illustrated in FIG. 2 for electroplating.

*Copper plating*

The zinc die castings were immersed with "current on" in a copper strike bath of the following composition:

|                                                   | Oz./gal. |
|---------------------------------------------------|----------|
| Sodium cyanide, NaCN                              | 3.5      |
| Copper cyanide, CuCN                              | 2        |
| Sodium carbonate, Na <sub>2</sub> CO <sub>3</sub> | 2        |
| Rochelle salts                                    | 2        |

Free sodium cyanide was maintained between 1.0 and 1.7 oz./gal. The temperature of the copper-strike bath was maintained between 122 and 130° F., and the work bar was agitated 15 ft./min. About 0.00005 inch (0.05 mil) of copper was deposited in 2 to 3 minutes at a current density of 60 amp./sq. ft. The parts were rinsed in cold water.

Copper plating was continued in a high-efficiency, bright-plating copper bath of the following composition:

|                                                     | Oz./gal. |
|-----------------------------------------------------|----------|
| Copper cyanide, CuCN                                | 11       |
| Potassium cyanide, KCN                              | 9.5      |
| Sodium cyanide (sulfide-free NaCN)                  | 6.0      |
| Potassium hydroxide, KOH                            | 3.0      |
| Potassium carbonate, K <sub>2</sub> CO <sub>3</sub> | 8.0      |

NOTE: Together with leveling agents, wetting agents, and porosity preventing agents.

Plating conditions were as follows:

|                         |                                                               |
|-------------------------|---------------------------------------------------------------|
| Temperature             | 172 to 180° F.                                                |
| Cathode current density | 42 amp./sq. ft.                                               |
| Agitation               | Work bar at 15 ft./min. plus air.                             |
| Anodes                  | Oxygen - free, high conductivity, oval-shaped, copper anodes. |
|                         |                                                               |

The plating time was predetermined for each part by employing duplicate samples, and depended on the specified thickness range required by the supplier for the significant recessed area.

*Duplex-nickel plating*

The freshly copper-plated parts are rinsed in warm water, dipped in a 10 percent sulfuric acid solution, rinsed in cold water, and nickel plated in a semibright-plating nickel bath having the following composition:

|                                                       |          |      |
|-------------------------------------------------------|----------|------|
| Nickel sulfate, NiSO <sub>4</sub> ·6H <sub>2</sub> O  | oz./gal. | 42.5 |
| Nickel chloride, NiCl <sub>2</sub> ·6H <sub>2</sub> O | oz./gal. | 5.8  |
| Boric acid, H <sub>3</sub> BO <sub>3</sub>            | oz./gal. | 5.9  |

<sup>1</sup> Optimum appearance is defined in terms of the number of minutes of electropolishing before porosity is observed. It is necessary to follow electropolishing with the required thicknesses of electrodeposits to facilitate this determination. Electropolishing time will ordinarily be between 0.25 and 8 minutes.

7  
 Wetting agent (2% solution Na lauryl sulfate) percent by volume 0.6  
 Leveling agent, coumarin lb./100 gal. 0.6 to 1.1

Plating conditions were as follows:

pH 4.0 to 4.4.  
 Agitation Work bar at 23 ft./min.  
 Anodes Carbon type, rolled, oval, 99+ percent nickel in cotton anode bags.  
 Temperature 126 to 130° F.  
 Cathode-current density 60 amp./sq. ft.  
 Plating time

10  
 15  
 20  
 25  
 30  
 35  
 40  
 45  
 50  
 55  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895  
 5900  
 5905  
 5910  
 5915  
 5920  
 5925  
 5930  
 5935  
 5940  
 5945  
 5950  
 5955  
 5960  
 5965  
 5970  
 5975  
 5980  
 5985  
 5990  
 5995  
 6000  
 6005  
 6010  
 6015  
 6020  
 6025  
 6030  
 6035  
 6040  
 6045  
 6050  
 6055  
 6060  
 6065  
 6070  
 6075  
 6080  
 6085  
 6090  
 6095  
 6100  
 6105  
 6110  
 6115  
 6120  
 6125  
 6130  
 6135  
 6140  
 6145  
 6150  
 6155  
 6160  
 6165  
 6170  
 6175  
 6180  
 6185  
 6190  
 6195  
 6200  
 6205  
 6210  
 6215  
 6220  
 6225  
 6230  
 6235  
 6240  
 6245  
 6250  
 6255  
 6260  
 6265  
 6270  
 6275  
 6280  
 6285  
 6290  
 6295  
 6300  
 6305  
 6310  
 6315  
 6320  
 6325  
 6330  
 6335  
 6340  
 6345  
 6350  
 6355  
 6360  
 6365  
 6370  
 6375  
 6380  
 6385  
 6390  
 6395  
 6400  
 6405  
 6410  
 6415  
 6420  
 6425  
 6430  
 6435  
 6440  
 6445  
 6450  
 6455  
 6460  
 6465  
 6470  
 6475  
 6480  
 6485  
 6490  
 6495  
 6500  
 6505  
 6510  
 6515  
 6520  
 6525  
 6530  
 6535  
 6540  
 6545  
 6550  
 6555  
 6560  
 6565  
 6570  
 6575  
 6580  
 6585  
 6590  
 6595  
 6600  
 6605  
 6610  
 6615  
 6620  
 6625  
 6630  
 6635  
 6640  
 6645  
 6650  
 6655  
 6660  
 6665  
 6670  
 6675  
 6680  
 6685  
 6690  
 6695  
 6700  
 6705  
 6710  
 6715  
 6720  
 6725  
 6730  
 6735  
 6740  
 6745  
 6750  
 6755  
 6760  
 6765  
 6770  
 6775  
 6780  
 6785  
 6790  
 6795  
 6800  
 6805  
 6810  
 6815  
 6820  
 6825  
 6830  
 6835  
 6840  
 6845  
 6850  
 6855  
 6860  
 6865  
 6870  
 6875  
 6880  
 6885  
 6890  
 6895  
 6900  
 6905  
 6910  
 6915  
 6920  
 6925  
 6930  
 6935  
 6940  
 6945  
 6950  
 6955  
 6960  
 6965  
 6970  
 6975  
 6980  
 6985  
 6990  
 6995  
 7000  
 7005  
 7010  
 7015  
 7020  
 7025  
 7030  
 7035  
 7040  
 7045  
 7050  
 7055  
 7060  
 7065  
 7

jecting the article to electrolytic polishing in an electrolytic cell in which the article is the anode, the electrolyte is comprised substantially of an aqueous alkali metal hydroxide solution in the amount between about 450 and 900 grams of alkali metal hydroxide, about 20 and 100 grams of zinc oxide and the trivalent chromic ion equivalent of about 1.5 and 3 grams of basic chromic sulfate per liter of solution maintained at a temperature between about 60 and 220° F., the cathode is magnetic coated, and the current passing between the anode and the cathode has a current density of between about 50 and 800 amperes per square foot and is maintained at a voltage of about 4 to 11 volts for a period of about 0.25 to 8 minutes, to polish the article and clean out any surface pores therein, rinsing the electrolyte from the electropolished article, acid dipping the electropolished article and subjecting the article to electroplating in an electroplating cell to plate the article and the electropolished exposed bottom of any surface pores thereon, until the desired composition and thickness of plate has been deposited on said article.

3. The method of reducing blistering and plating failures on electroplated cast zinc base articles which comprises electropolishing said articles in an electrolytic cell in which the article is the anode, the electrolyte is comprised substantially of an aqueous solution of sodium hydroxide in the amount between about 572 and 763 grams per liter and about 20 and 100 grams of zinc oxide and the trivalent chromic ion equivalent of about 1.5 and 3 grams of basic sulfate per liter maintained at a temperature between about 73 and 100° F., the cathode is a conducting material, and the current passing between the anode and the cathode has a current density of between about 100 and 200 amperes per square foot and is maintained at a voltage of about 8 for a period of about 0.75 to 8 minutes, whereby the surface of said article is evened, corners are rounded out and pits are freed of foreign matter to provide clean metal over the entire surface of said article and thereafter subjecting the article to electroplating in electroplating cells to plate the article over the electropolished surface and the bottom of said pits, until the desired composition and thickness of plate has been deposited on said article.

4. The method of reducing blistering and plating failures on electroplated cast zinc base articles which comprises electropolishing said articles in an electrolytic cell in which the article is the anode, and the electrolyte is comprised substantially of about 600 to 700 grams per liter of an aqueous sodium hydroxide solution, containing about 20 to 30 grams per liter zinc oxide and about 1.5 to 3 grams per liter of basic chromic sulfate maintained at a temperature between about 80 and 95° F., the cathode is a magnetic coated material, and the current passing between the anode and the cathode has a current density

of between about 100 and 200 amperes per square foot and is maintained at a voltage of about 8 for a period of about 0.75 to 1.5 minutes, whereby the surface of said article is evened, corners are rounded out and pits are freed of foreign matter to provide clean metal over the entire surface of said article and thereafter subjecting the article to electroplating in electroplating cells to plate the article over the electropolished surface and the bottom of said pits, until the desired composition and thickness of plate has been deposited on said article.

5. The method of reducing blistering and plating failures in electroplated cast zinc base die castings which comprises subjecting the casting to electropolishing in an electrolytic cell in which the casting is the anode and the electrolyte comprised of an aqueous solution of an alkali metal hydroxide of the group consisting of sodium and potassium hydroxides in an amount between about 600 to 700 grams per liter, zinc oxide in an amount between about 20 and 30 grams per liter and basic chromic sulfate in an amount of about 2 grams per liter, maintained at a temperature between about 75 to 100° F., the cathode is a conducting material and the current passing between the anode and the cathode has an anode current density of 100 to 200 amps/sq. ft. for a period of about 0.75 to 2 minutes after the castings have been buffed and before electroplating to clean the buffing compounds out of depressions in the castings and round out the corners of said depressions, and after electropolishing said buffed castings, rinsing, acid dipping and electroplating said castings.

6. The method of electropolishing cast zinc base articles which comprises, subjecting the article to electropolishing in an electrolytic cell in which the article is the anode, the electrolyte is comprised substantially of an aqueous alkali metal hydroxide, between about 20 and 100 grams of zinc oxide and the trivalent chromic ion equivalent of between about 1.5 and 3 grams of basic chromic sulfate per liter of solution, maintained at a temperature between about 60 and 220° F., the cathode is a conducting material, and the current passing between the anode and the cathode has a current density of between 50 and 800 amperes per square foot and is maintained at a voltage of about 8 for a period of about 0.25 to 8 minutes, to polish the article and clean out any surface pores therein.

#### References Cited by the Examiner

Graham: "Electroplating Engineering Handbook"; 2nd edition, 1962; pages 68-82, 107-125, 186, 190-193, 198. Plating, volume 45, 1027-1037 (October 1958).

WINSTON A. DOUGLAS, Primary Examiner.

MURRAY TILLMAN, Examiner.